

## 1

3,481,904  
COMPLEX-FORMING POLY-SCHIFF'S BASES  
Ernst Bayer, Melanchthon-Strasse 33,  
Tuebingen, Germany

No Drawing. Filed Aug. 26, 1966, Ser. No. 575,239  
Claims priority, application Germany, Oct. 28, 1965,  
B 84,286

Int. Cl. C08g 9/06; C22b 11/04  
U.S. Cl. 260—72

3 Claims

### ABSTRACT OF THE DISCLOSURE

A poly-Schiff's base consisting essentially of recurring units of the formula



wherein  $n$  is an integer of 10–2000, and a process for producing the same by condensing 1,4-diamino-2,5-dimercaptobenzene and at least a stoichiometric amount of glyoxal, effecting the reaction in an aqueous solution at a temperature of about 40–90°C.

This invention relates to a poly-Schiff's base which can be used as a specific complex former or ion exchanger for gold.

It is known [cf. E. Bayer et al., "Angewandte Chemie" 76 76 (1964)] that it is possible, by polycondensing 2,5-diaminothiophenol and glyoxal, to obtain a polycondensate probably corresponding to Formula 1:



This material is able to form complexes with metal ions, particularly those of the first and second subsidiary groups of the periodic system, and to release them again.

It has now been found that improved polycondensates can be obtained by polycondensing 1,4-diamino-2,5-dimercaptobenzene and glyoxal in aqueous solution at temperatures in the range from 40 to 90°C. The following general formula may be attributed to these polycondensates.



In this formula,  $n$  is a number greater than 10 and may be as high as 2,000, preferably in the range of about 20 to about 200.

To prepare this polycondensate, the glyoxal is preferably used in an amount equivalent to that of the 1,4-diamino-2,5-dimercaptobenzene or in an excess of up to 10 times the stoichiometrically necessary quantity.

The polycondensate according to the invention is a complex-former which is practically specific for gold (III) ions and is therefore suitable for isolating gold (III) ions from dilute solutions, even if these solutions contain other metal ions.

The material only combines with metals of the first and second subsidiary groups of the periodic system, gold being very much preferred as shown by the following

## 2

table. This table illustrates the ability of the metals of the first and second subsidiary groups of the periodic system to combine with the polycondensates of this invention.

|                  |       | Capacity               |                                      |
|------------------|-------|------------------------|--------------------------------------|
|                  |       | Percent of theoretical | G. atom/100 g. of poly-Schiff's base |
| Ion:             |       |                        |                                      |
| Zn <sup>2+</sup> | ..... | 0                      | 0                                    |
| Cd <sup>2+</sup> | ..... | 0                      | 0                                    |
| Hg <sup>2+</sup> | ..... | 23.7                   | 0.12                                 |
| Cu <sup>2+</sup> | ..... | 5.5                    | 0.02                                 |
| Ag <sup>2+</sup> | ..... | 31.4                   | 0.15                                 |
| Au <sup>3+</sup> | ..... | 101                    | 0.5                                  |

The ability of the complex-former to combine with gold is extremely high and better than that of all the hitherto known complex-formers. Theoretically it is equivalent to 2 gram-atoms of gold per molecule unit, i.e., 394 g. of gold per 388 g. of complex-former. This capacity is also achieved in practice.

In addition, it is possible to remove the gold which has accumulated on the complex-former, for example by treatment with an acid, so that the polycondensate according to the invention can be used as an ion-exchanger specific for gold (III) ions.

The gold is advantageously removed from the complex-former by treatment with hydrochloric acid, for example, by shaking with 4 N hydrochloric acid. The acid is preferably contacted with the complex for a prolonged contact time of up to 12 hours.

Any metal residues still adhering to the complex-former after such a treatment can be removed by treatment with sodium or potassium cyanide. The material may then be used again to absorb gold.

These methods of recovering the gold result in concentrated gold (III)-salt solutions, more specifically in complex salt solutions. The metallic gold has to be recovered from the solutions obtained according to known methods.

In another method of recovering the gold the charged complex-forming poly-Schiff's base is heated to a temperature above about 250 and up to 600°C. The organic material is destroyed in this heating process and the gold is recovered in metallic form. As the poly-Schiff's base has a very high capacity of absorbing gold, the amounts of this polymer used are rather small. Therefore, destroying these absorbing agents may be more economical than as expensive recovering process.

The polycondensate is insoluble in the conventional organic solvents, for example, alcohols, ethers, dimethylformamide, acetone, chloroform, benzene and hydrocarbons, and also in water. It is resistant to weak acids and weak alkaline liquors.

### EXAMPLE 1

#### Preparation of the poly-Schiff's base from 1,4-diamino-2,5-dimercaptobenzene and glyoxal

3.5 g. (0.014 mol) of thoroughly purified 1,4-diamino-2,5-dimercaptobenzene dihydrochloride were dissolved with continuous stirring in 70 ml. of distilled water through which nitrogen was bubbled. To prepare the free diamine, 14 ml. of a 12% by weight soda solution were added dropwise to the solution in a stream of nitrogen so that the pH-value of the mixture was about 7. Following complete neutralisation, the brownish-green solution was heated to 60°C. in a paraffin bath, after which 8.8 g. (0.06 mol) of 40% by weight aqueous glyoxal solution were added dropwise to it at this temperature in a stream of nitrogen. After all the glyoxal solution had been added, the product was stirred for another half hour at 60°C. and cooled to 0°C., and the precipitated brownish-green product suction-filtered. It was briefly boiled in 50 ml. of boiling water, suction-

filtered again and washed with 20 ml. of hot water. The polycondensate was dried over diphosphorus pentoxide for 20 hours at room temperature/14 mm. Hg. The poly-Schiff's base was obtained as a brownish-green fine-grained powder. Yield=2.4 g. (86% of the theoretical).

To remove acid-soluble components, the poly-Schiff's base was stirred for 20 hours at room temperature in 0.1 N hydrochloric acid. The product was then suction-filtered and successively washed three times with 10 ml. of distilled water, 10 ml. of methanol and 10 ml. of ether and then dried over diphosphorus pentoxide at 20° C./14 mm. Hg until its weight was constant.

#### EXAMPLE 2

1 ml. of a 0.01 molar solution of zinc sulphate, 1 ml. of cadmium acetate, 1 ml. of mercury (II) acetate, 1 ml. of copper acetate and 1 ml. of tetrachloro-gold (III)-acid, were mixed together and made up to 1 litre with distilled water. 1 g. of poly-Schiff's base, obtained as in Example 1, was added to this solution which was then shaken for 12 hours at room temperature. The macromolecule was then filtered off, after which the metal contents both of the filtrate and of the macromolecule are determined. Whereas the gold quantitatively combined with the macromolecule, the copper (II)-, cadmium and zinc ions remained quantitatively in the solution. Only about one tenth of the mercury originally introduced also combined. The macromolecule was found to have combined with 1.92 mg. of gold (98%), 0.22 mg. of mercury (11%) and less than 0.002 mg. each of copper, cadmium and zinc.

50 mg. of gold-containing poly-Schiff's base were shaken for 12 hours at 20° C. with 300 ml. of 0.1 N hydrochloric acid. 65% of the gold was released to the solution under these conditions.

10  
5

To remove the remaining gold, the product was shaken for 3 hours with 100 ml. of a 0.01 N sodium cyanide solution.

I claim:

1. Poly-Schiff's base consisting essentially of recurring units of the formula



15 where  $n$  is an integer of 10-2,000.

2. The compound of claim 1 wherein  $n$  is an integer of 20-200.

20 3. Process for producing poly-Schiff's bases which comprises condensing 1,4-diamino-2,5-dimercaptobenzene and at least a stoichiometrical amount of glyoxal, effecting the reaction in an aqueous solution at a temperature of about 40-90° C.

#### References Cited

##### UNITED STATES PATENTS

2,412,855 12/1946 Auten et al.  
2,653,089 9/1953 Brooke.

25 WILLIAM H. SHORT, Primary Examiner

L. M. PHYNES, Assistant Examiner

30 U.S. CL. X.R.

35 75-118; 260-2.2, 67.5, 566